

Sept. 13, 1932.

E. H. BUNCE

1,877,123

PRODUCING COKE AGGLOMERATES

Filed July 30, 1929

Fig. 1,



Fig. 2.



INVENTOR  
EARL H. BUNCE

BY

*James, Davis, Marvin Edmonds*  
ATTORNEYS

## UNITED STATES PATENT OFFICE

EARL H. BUNCE, OF PALMERTON, PENNSYLVANIA, ASSIGNOR TO THE NEW JERSEY ZINC COMPANY, OF NEW YORK, N. Y., A CORPORATION OF NEW JERSEY

## PRODUCING COKE AGGLOMERATES

Application filed July 30, 1929. Serial No. 382,273.

This invention relates to the production of coked agglomerates of mixed metalliferous material and carbonaceous material, and has for its object the provision of certain improvements in the preparation and coking of such agglomerates. While the invention, in its broad aspect, aims to provide certain improvements in the production of coked agglomerates of mixed metalliferous and carbonaceous materials, it more especially contemplates the production of coked agglomerates of mixed zinciferous material and carbonaceous material, and will hence be herein described with particular reference to the production of such coked agglomerates.

Coked agglomerates of mixed zinciferous and carbonaceous materials constitute a peculiarly advantageous charge for the smelting or reduction of the zinciferous material, particularly in vertical zinc distillation retorts. In the preparation of such coked agglomerates for vertical retort smelting, the major consideration is the strength of the residue after the zinc has been eliminated—briefly characterized as residue strength. Thus, the coked agglomerates must possess sufficient strength to pass progressively through the vertical retort without breaking down or sanding and to provide a residue of sufficient strength to prevent disintegration by crumbling, rupturing or abrading. Hence, it is always necessary to know the residue strength of the coked agglomerates in order to determine whether or not the agglomerates can be satisfactorily smelted in a vertical retort.

In the preparation of these coked agglomerates, it is customary to first separately crush the zinciferous material (e. g. zinc ore) and the carbonaceous material (e. g. coal) and then to knead these materials together in a Chilean mill or edge-runner (frequently called a chaser) to form a mixture that is suitable for agglomerating. The necessary intimate contact of the ore and coal particles for both reduction and ultimate residue strength is advantageously promoted by appropriate graded sizing of the ore and coal as described in the copending patent application of Thomas C. Routson and myself, Serial No. 301,709, filed August 23, 1928. If

necessary, a conditioning agent or a binder, such as sulfite liquor, tar, pitch, or the like, may be added during the treatment in the edge-runner. The mixture thus prepared in the edge-runner is next agglomerated, usually by briquetting, and then coked at temperatures insufficient to cause any substantial loss of zinc.

The purpose of coking the agglomerate is to utilize the coke bond for holding the ore and coal particles together. In coked agglomerates for vertical retort smelting, it is very desirable, if not essential, that the coke bond be a cellular or lattice structure intimately bonded with and enveloping the particles of zinc ore, and of sufficient strength to prevent both splitting up of the agglomerates during coking and disintegration during the subsequent smelting or reduction. The active bonding or coking constituent of the agglomerate mixture (zinciferous and carbonaceous materials) is the bituminous coal or equivalent coking agent including in the mixture. The amount of bituminous coal, or equivalent coking agent, necessary to give satisfactory residue strength is dependent entirely upon the nature of the coal or equivalent coking agent used. It has been found advantageous to include in the agglomerate mixture, as part or all of the bituminous coal required for coking, a certain amount of a free-flowing coal as described in the aforementioned patent application. These and economic considerations determine the character of the carbonaceous material of the agglomerate mixture, and usually make it desirable in practice to make up the carbonaceous material of a mixture of coals.

The method used in coking the agglomerates is dependent, to a very large extent at least, upon the amount and nature of the bituminous coal constituting all or part of the carbonaceous material of the agglomerate mixture. In certain localities, it is desirable, for economic reasons, to use as little bituminous coal as possible. In other localities it may be economically advantageous to use all bituminous coal. The present invention is concerned primarily with the provision of an improved method of coking these ore and

coal agglomerates and is particularly applicable in those localities where it is desirable to use the minimum amount of bituminous coal or equivalent coking agent.

- 5 The method of coking contemplated by the invention may be characterized as "rapid coking", since the aim is to form a shell of coke on the agglomerate as promptly as possible. This prompt formation of a shell of coke on the agglomerate is effected by initially subjecting the agglomerate to a high temperature rapid coking treatment so that a substantial layer of coke forms at the surface of the agglomerate in a relatively short time 10 interval and while the main inner mass of the agglomerate remains substantially unaltered. The high temperature heat treatment is then continued until the entire agglomerate is coked. Thus, in carrying out 15 the invention, the appropriately prepared agglomerates of mixed metalliferous and carbonaceous materials are subjected to such a rapid initial application of heat as to promptly form a shell of coke on the surface 20 of each agglomerate. After the shell of coke has formed on the surface, the heat penetrates further into the agglomerate and coking progresses until the whole agglomerate is 25 coked.
- 20 The rapid initial heating of the agglomerates may be effected in any appropriate manner. The ideal practice involves the initial application to each agglomerate of heat at or slightly above the requisite temperature 30 for coking, and in sufficient quantity to immediately form a shell of coke on the agglomerate. While such a condition of heat treatment is difficult of realization under practical operating conditions, it should be 35 closely approximated as possible if the optimum advantages characteristic of the invention are to be attained. Accordingly, in practice, a source of heat at or above the temperature required for coking is applied to 40 the body of agglomerates to be coked so as to heat the surface layer of each agglomerate to the coking temperature as promptly as possible. Thus, it may be said that the starting 45 of the coking operation is at or above the finishing temperature of coking, in contradistinction to those coking practices in which the material to be coked is gradually raised to the requisite coking temperature. Furthermore, in the practice of the invention, this 50 high temperature heat, which is initially applied to the agglomerates, must be available in sufficient quantity to rapidly form the contemplated shell of coke on the agglomerate and to continue and complete the coking of 55 the entire agglomerate.

The agglomerates may be subjected to the coking operation without preliminary drying or heating. By the customary mode of preparation, the agglomerates contain about 65 6 to 12% by weight of moisture, and are

therefore relatively moist. It is a characteristic feature of the present invention that these relatively moist agglomerates may be immediately subjected to the highest temperature required for coking. It is advantageous 70 to transfer the agglomerates direct from the agglomerating apparatus, for example a briquetting press, to the coking apparatus, whereby the moist agglomerates are immediately subjected to the heating medium at a temperature at or above the finishing 75 temperature of coking.

The coking operation is preferably conducted by direct contact of a gaseous heating medium with the agglomerates. This 80 is desirable since it insures the contemplated rapid as well as uniform heating of the surface of the agglomerates to the requisite coking temperature, and at the same time permits economic and efficient transfer of 85 heat from the heating medium to the agglomerates. The charge of agglomerates should be exposed to the heating medium in the form of a relatively shallow or thin body through which a large volume of the heating 90 gas passes at high velocity.

Any appropriate source of heating gas (inert to the charge under the conditions of coking) may be used in coking the agglomerates by direct heating. The heating gas 95 must be substantially devoid of oxidizing influences. During the early or formative stage of coking, oxygen or oxidizing influences deleteriously affect the coking constituent or fraction of the agglomerate, and it 100 is particularly important that this stage of the coking operation be conducted in the absence of such oxidizing influences. Oxidizing influences should also be avoided during the later stages of the coking operation, since 105 they tend to consume the coke.

The heating gas may be producer gas, illuminating gas, oil gas, natural gas, coke-oven gas, water gas, and similar fuel gases, extraneously heated where necessary. The 110 combustion gases resulting from burning such fuel gas, oil or coal (or similar solid carbonaceous fuel) may be used as the heating gas. Such combustion gases may be the exhaust gases from a contiguous thermic 115 operation, when using such combustion gases, it may be desirable or even necessary to add a small quantity of unburned fuel gas to the combustion gases in order to react with or neutralize any oxidizing gases, such as excess oxygen, therein. Other inert gases, such as nitrogen, superheated steam, and the like, may also be used as the direct heating gas.

The heating gas may as a result of its 120 method of production or previous use be of appropriate temperature for the coking operation. Where the gas is too hot for the contemplated coking operation, it should be appropriately cooled, as for example, by steam, water, or the like. If the heating gas 125

is not of a sufficiently elevated temperature for the coking operation, it must be appropriately heated. This may be advantageously accomplished by recuperation, or by regeneration, or by adding thereto an appropriate volume of a hotter gas, or by combust-  
ing some of the gas itself or a combustible constituent added thereto for the purpose.

When the heating gas contains or is itself a fuel gas, it is frequently advantageous to combust the gas exiting from the charge undergoing coking, and to utilize the resulting heat of combustion for heating the gas-exiting side of the charge. This may be accomplished by adding oxygen to the gas exiting from the charge and supplying the resulting heat of combustion, preferably by radiation, to the gas-exiting side of the body of charge undergoing coking. In this manner a certain compensation is effected for the natural drop in temperature of the heating gas in passing through the body of charge undergoing coking.

When, in practicing the present invention, the coking operation is carried out by direct contact of the agglomerates with a gaseous heating medium, the heating gas should be of such temperature that the surface of each agglomerate is rapidly heated to 800° C. or higher. I have obtained very satisfactory results with a heating gas entering the body of agglomerates undergoing coking at a temperature of from 800 to 1000° C. and exiting from the body of agglomerates at a temperature of from 700 to 800° C., but not lower than 550° C. The drop in temperature of the heating gas in passing through the agglomerates may be minimized by the extraneous application of heat to the gas-exiting side of the body of agglomerates, as for example in the manner hereinbefore described. The coking of the agglomerates, under the preferred conditions herein described, will take from 30 to 90 minutes, depending upon the size of the individual agglomerates, the depth or width of the body of charge, and the volume and velocity of the heating gas.

The coked agglomerates are preferably transferred without substantial loss of heat after coking to the zinc distillation retort. Where this practice is not followed and it is necessary to store and hence cool the coked agglomerates before smelting, they should be cooled, directly upon discharge from the coking operation, under reducing or non-oxidizing conditions, such for example as in an atmosphere of non-oxidizing or reducing gas or in a mass of carbonaceous material, or in receptacles, such as sealed cans, from which air is excluded.

While I prefer, in practicing the invention, to coke by direct contact with a gaseous heating medium, the requisite heat for coking may be supplied to the agglomerates in any other appropriate manner, provided, of

course, that the supply of heat is adequate to effect the rapid surface coking of the agglomerates characteristic of the invention.

Any suitable apparatus may be employed for exposing a shallow or thin body of agglomerates to the heating medium. Thus, the charge of agglomerates undergoing coking may be supported on a stationary or moving hearth or perforated grate, or may be supported within a vertically disposed or inclined chamber operated intermittently or continuously, but preferably arranged to permit progressive movement of the agglomerates therethrough by the action of gravity. The invention may very advantageously be carried out in the cross-current vertical coking furnace described in my co-pending patent application, Serial No. 391,825 filed September 11, 1929.

Merely by way of illustration, I give the following specific example of the practice of the invention. The zinciferous material and coal were of the graded size and were mixed and briquetted in accordance with the practice described in the aforementioned Routson and Bunce application Serial No. 301,709. Using roasted and sintered flotation concentrates, the practice described in my co-pending application Serial No. 319,735, filed November 15, 1928 was followed. The composition of the agglomerate mixture was as follows:

|                                               | Per cent<br>by weight |
|-----------------------------------------------|-----------------------|
| Zinciferous material                          | 60                    |
| Anthracite dust coal                          | 20                    |
| Free-flowing coal (high resinous bodied coal) | 20                    |

The mixture contained 10% moisture based on the dry weight of the ore and coal. From 1 to 3% of sulphite liquor was added during mixing as a temporary binder and also for its beneficial action as a wetting agent.

The briquetted mixture, without drying, was coked in the cross-current vertical coking furnace hereinbefore mentioned, the heating gas entering one side of the body of briquettes undergoing coking at a temperature of about 900° C. and exiting from the other side at a temperature of about 700° C. The time required for the complete coking operation was about 45 minutes. To produce the desired shell of coke on each briquette in the shortest time possible, it is necessary to pass as large a volume of heating gas as possible through that region where the coke shell is being formed. After the coke shell is formed, the interior of the briquette is coked by the continued passage of a large volume of the heating gas through the charge undergoing coking. The resulting coked agglomerates were subsequently smelted in a vertical retort in accordance with the practice disclosed in U. S. patent of Breyer and Bunce No. 1,712,132 and satisfactorily retained their

agglomerated form without substantial deformation or breaking down throughout the entire reduction period.

It is characteristic of the invention that the agglomerates are heated from room temperature to the effective coking temperature in as short a time interval as possible. This initial rapid heating produces a shell of coke which prevents excessive losses from abrasion and is strong enough to withstand the internal forces developed by subsequent drying and coking, which tend to rupture the agglomerates. This shell of coke also enables the agglomerates to withstand the load of the column of agglomerates above it, without deformation. A temperature of 900° C. at the inlet and 650° C. (but not lower than 550° C.) at the outlet of the body of agglomerates undergoing coking, with direct heating, produces the desired shell of coke. The optimum conditions for uniformly producing the shell of coke throughout the body of agglomerates occur with the lowest temperature drop from the gas inlet to the gas outlet. This condition limits the width, or depth, of the body of agglomerates in that region where the coke shell is being formed. I have found a width of about 16 inches very satisfactory in the aforementioned cross-current vertical coking furnace, but this width may be enlarged with higher temperatures and greater gas volumes, provided that an adequate volume of heating gas can be made to pass through the agglomerates without too great a drop in temperature and pressure.

The following table is a log of a coking operation conducted in accordance with the principles of the invention. The agglomerate mixture was of substantially the same composition as described in the preceding example, and was briquetted into four inch loaf briquettes, and the briquettes were charged directly into the coking furnace. This furnace consisted of a chamber containing horizontally disposed grate bars and a flue for conducting the heating gas to the chamber below the grate bars. The briquettes were placed on the grate bars and the heating gas from the flue passed upwardly through the bed of briquettes and was exhausted to the atmosphere. The heating gas was delivered to the briquettes at a temperature of 900° C. The coking operation was completed in 30 minutes.

Log of coking operation

| Sample number | Minutes after charging | Appearance of briquette when removed and broken in half |
|---------------|------------------------|---------------------------------------------------------|
| 1             | 5                      | 1/4" coke shell—center wet.                             |
| 2             | 10                     | 1/4" coke shell—center wet.                             |
| 3             | 15                     | 1/4" coke shell—center plastic.                         |
| 4             | 20                     | Entire briquette solid, but volatile being removed.     |
| 5             | 25                     | Entire briquette solid, but volatile being removed.     |
| 6             | 30                     | Entire briquette solid; all volatile removed            |

It is characteristic of the invention that

within a few minutes after charging a substantial layer of coke forms at the surface of the agglomerate while the core is still in its original moist condition. This layer of coke progressively moves towards the center until ultimately the entire agglomerate is coked. Complete coking of the agglomerate is accomplished in a relatively short interval of time with little or no danger of disrupting the agglomerate during the coking operation. At the end of the coking period, the agglomerate is a homogeneous piece of coke with no indication of layers or zones having been formed. The coke is free from breeze and is dense and strong.

The coking method of the invention is particularly adapted for the economic production of coke and residue strengths. While the invention is of particular advantage for coking agglomerates in which the carbonaceous material consists of a mixture of a free-flowing coal and anthracite or coke fines, it may be practiced with advantage where the carbonaceous material consists of a blend of bituminous coals including some free-flowing coal, and where the carbonaceous material is a bituminous coal possessing of itself such properties as adapt it for this method of coking. While it is our preferred practice to effect the contemplated coking action by bituminous coal, other equivalent carbonaceous coking agents may be substituted in whole or in part for the bituminous coal, such as tar, pitch, and the like. Anthracite or coke fines are included in the agglomerate mixture primarily for the purpose of imparting adequate residue strength, and where the use of these fines is uneconomical, other materials not affected by the prevailing conditions of reduction, such as slate coal, sand, saggers, etc., may be substituted in whole or in part for such fines.

In the foregoing discussion I have particularly described the invention in connection with the production of coked agglomerates of mixed zinciferous and carbonaceous materials. Such coked agglomerates, while peculiarly adapted for smelting in vertical retorts, may be treated by any other appropriate metallurgical operation. Moreover, the invention is not restricted to zinciferous materials, but may be practiced with advantage in producing coked agglomerates of any other metalliferous material.

The novel features of the invention will be best understood from the following description taken in conjunction with the accompanying drawings, in which

Fig. 1 is a sectional elevation of a coking furnace adapted for a practice of the invention; and

Fig. 2 is a cross section of the furnace of Fig. 1 on the section line 2—2.

Referring to Figs. 1 and 2 of the drawing, the furnace comprises a brickwork structure

5, of oval horizontal section, having a gas inlet flue 6 and a gas outlet flue 7. Clean-out openings 20 are provided in the curved ends of the structure 5. A relatively narrow coking chamber 8 is built midway between the ends of the structure 5, thereby providing on one side a gas distributing laboratory or chamber 9 communicating with the inlet 6 and on the other side a similar laboratory or chamber 10 communicating with the outlet 7. One side wall 12 of the coking chamber is substantially vertical, while the other side wall 13 is slightly inclined outwardly so that the cross sectional area of the chamber increases from the top to the bottom. Both side walls of the coking chamber are permeable to the passage therethrough of gas in considerable volume. This permeability is preferably provided by uniformly distributed openings 20 or slots in each side wall.

In the coking chamber illustrated in Figs. 1 and 2 of the drawing, the vertical side wall 12 is built up of superposed tiles or plates having uniformly distributed slots. These tiles may be made of refractory material, such as silicon carbide alone or mixed with clay, or of temperature resistant metal alloys, such as alloys of iron, chromium and nickel. The inclined wall 13 is built of louvers positioned so that the gas stream leaving the coking chamber is directed upwardly into the gas-exiting chamber 10. This louver construction minimizes the possibility of dust and broken pieces of agglomerates lodging in and choking the openings on the gas-exit side of the coking chamber.

The upper end of the coking chamber passing through the roof of the furnace structure 5 has a water jacket 21. A charging extension or hopper 22 provided with a swinging gate 23 is mounted above the water jacket. A pipe 24 connects the extension 22 with the gas-exiting chamber 10, which is adapted to remove by suction oxidizing air entrapped in the charge hopper 22 and also to remove by suction any heating gases that may rise upwardly through the column of agglomerated charge materials into the hopper 22.

A discharging device consisting of an inclined chute 25 and a rotatably mounted cylinder 26 is operatively associated with the lower end of the coking chamber 8. The lower end of the chute is closed by a pivotally mounted gate 27 biased to its closed position by a counterweight 28. A pipe 29 connects the lower end of the chute with the gas-exiting chamber 10.

When the furnace is in operation, the coking chamber 8 is filled with agglomerates undergoing coking. Periodically, an appropriate amount of coked agglomerates is withdrawn from the chamber by opening the gate 27 and rotating the cylinder 26, and simultaneously a corresponding amount of fresh agglomerates is introduced into the hopper 22. The

coking chamber is thereby maintained full and the green or fresh agglomerates are charged with a minimum drop or fall.

The heating gas for coking is introduced through the gas inlet 6. Any appropriate source of heating gas (inert to the charge under the conditions of coking) may be used. Thus, the heating gas may be producer gas, illuminating gas, oil gas, natural gas, coke oven gas, water gas, and similar fuel gases, extraneously heated when necessary. The combustion gases resulting from burning such fuel gases, oil or coal (or similar solid carbonaceous fuel) may be used as the heating gas. Such combustion gases may be the exhaust gases from a contiguous thermic operation. When using such combustion gases, it may be desirable or even necessary to add a small quantity of unburnt fuel gas to the combustion gases in order to react with or neutralize any oxidizing gases, such as excess oxygen therein. Other inert gases, such as nitrogen, superheated steam, and the like, may also be used as the heating gas.

The heating gas must be substantially devoid of oxidizing influences. During the early or formative stage of coking, oxygen or oxidizing influences deleteriously affect the coking constituent or fraction of the agglomerate, and it is particularly important that this stage of the coking operation be conducted in the absence of such oxidizing influences. Oxidizing influences should also be avoided during the later stages of the coking operation since they tend to consume the coke.

The heating gas may as a result of its method of production or previous use be of appropriate temperature for the coking operation. Where the gas is too hot for the contemplated coking operation, it should be appropriately cooled as, for example, by steam, water or the like. If the heating gas is not of a sufficiently elevated temperature for the coking operation, it must be appropriately heated. This may be advantageously accomplished by recuperation, or by regeneration, or by adding thereto an appropriate volume of a hotter gas, or by combusting some of the gas itself or a combustible constituent added thereto for the purpose.

The heating gas enters the chamber 9 and is distributed through the openings of the vertical wall 12 into the coking chamber 8. The gas flows transversely through the body of agglomerates in the coking chamber and out through the openings in the sloping side wall 13 into the chamber 10 and to the gas outlet 7. The heating gas may be forced through the furnace, but is preferably drawn through by suction fans communicating with the gas outlet 7.

Some air unavoidably enters the hopper 22 during the charging operations. The deleterious effect of this air is minimized by the

provision of the pipe 24 which serves to suck the air from the hopper into the gas-exiting chamber 10. Even when the swinging gate 23 is closed, some air is likely to leak into the charging hopper, and such air is likewise drawn through the pipe 24 into the chamber 10. Similarly, the pipe 29 draws any air entering the discharge chute 25 into the chamber 10. The draft created by the exiting gases in the flue 7 establishes a sufficient suction in the pipes 24 and 29 to inhibit the flow into the active coking zone of the chamber 8 of any oxidizing gas resulting from the entrance of air through either the charging or discharging device. Where the heating gas is forced through the furnace (instead of drawn through by suction as in my preferred practice), the pipes 24 and 29 are omitted, since they would be inoperative in that case.

20 I claim:

1. The method of producing coked agglomerates which comprises preparing and agglomerating a mixture of metalliferous material and an appropriate coking agent, subjecting the agglomerates to a coking operation in which the agglomerates are initially heated by direct contact with a gaseous heating medium passed therethrough in sufficient volume and at a sufficiently high temperature to promptly form a shell of coke on each agglomerate, and continuing the heating of the agglomerates until coking thereof is completed.

25 2. The method of producing coked agglomerates which comprises preparing and agglomerating a mixture of metalliferous material and carbonaceous material, subjecting the agglomerates to a coking operation in which the agglomerates are initially heated by direct contact with a gaseous heating medium introduced into the agglomerates at a temperature at least as high as the effective coking temperature and leaving the agglomerates at a temperature not less than 550° C. and thereby promptly forming a shell of coke on each agglomerate, and continuing the heating of the agglomerates until coking thereof is completed.

30 3. The method of producing coked agglomerates which comprises preparing and agglomerating a mixture of metalliferous material and carbonaceous material, subjecting the agglomerates with a substantial moisture content to a coking operation in which the agglomerates are initially heated by direct contact with a gaseous heating medium passed therethrough in sufficient volume and at a sufficiently high temperature to promptly form a shell of coke on each agglomerate, and continuing the heating of the agglomerates until coking thereof is completed.

35 4. The method of producing coked agglomerates which comprises preparing and agglomerating an intimate mixture of zinc-

iferous material and carbonaceous material, subjecting the agglomerates to a coking operation in which the agglomerates are initially heated by direct contact with a gaseous heating medium passed therethrough in sufficient volume and at a sufficiently high temperature to promptly form a shell of coke on each agglomerate, and continuing the heating of the agglomerates until coking thereof is completed.

70 5. The method of producing coked agglomerates which comprises preparing and agglomerating an intimate mixture of zinciferous material and carbonaceous material, subjecting the agglomerates to a coking operation in which the agglomerates are initially heated by direct contact with a gaseous heating medium introduced into the agglomerates at a temperature at least as high as the effective coking temperature and leaving the agglomerates at a temperature not less than 550° C. and thereby promptly forming a shell of coke on each agglomerate, and continuing the heating of the agglomerates until coking thereof is completed.

75 6. The method of producing coked agglomerates which comprises preparing and agglomerating an intimate mixture of zinciferous material and carbonaceous material, subjecting the agglomerates with a substantial moisture content to a coking operation in which the agglomerates are initially heated by direct contact with a gaseous heating medium passed therethrough in sufficient volume and at a sufficiently high temperature to promptly form a shell of coke on each agglomerate, and continuing the heating of the agglomerates until coking thereof is completed.

80 7. The method of producing coked agglomerates which comprises preparing and agglomerating an intimate mixture of zinciferous material and carbonaceous material, subjecting said agglomerates to a coking operation in which the agglomerates are initially heated by direct contact with a gaseous heating medium passed therethrough in sufficient volume and at a sufficiently high temperature to promptly form a shell of coke on each agglomerate, and continuing the heating of the agglomerates until coking thereof is completed and thereby producing coked agglomerates possessing adequate residue strength when subjected to vertical retort smelting.

85 8. The method of producing coked agglomerates which comprises preparing and agglomerating an intimate mixture of zinciferous material and carbonaceous material, subjecting said agglomerates to a coking operation in which the agglomerates are initially heated by direct contact with a gaseous heating medium introduced into the agglomerates at a temperature not lower than 800° C. and leaving the agglomerates at a temperature not less than 550° C. and thereby promptly form-

- ing a shell of coke on each agglomerate, and continuing the heating of the agglomerates until coking thereof is completed and thereby producing coked agglomerates possessing adequate residue strength when subjected to vertical retort smelting.
9. The method of producing coked agglomerates which comprises preparing and agglomerating an intimate mixture of zinciferous material and carbonaceous material capable when appropriately coked of producing coked agglomerates possessing satisfactory residue strength for vertical retort smelting, subjecting said agglomerates with a moisture content of about 6 to 12% on the dry weight thereof to a coking operation characterized by an initial application of heat to the agglomerates at a temperature at or above the requisite coking temperature and thereby promptly forming a shell of coke on each agglomerate, and continuing the application of heat to the agglomerates until the entire mass of each agglomerate is heated to the requisite coking temperature.
- 25 10. The method of producing coked agglomerates which comprises preparing and agglomerating an intimate mixture of zinciferous material and carbonaceous material capable when appropriately coked of producing coked agglomerates possessing satisfactory residue strength for vertical retort smelting, subjecting said agglomerates with a moisture content of about 6 to 12% on the dry weight thereof to a coking operation in which the agglomerates are initially heated by direct contact with a gaseous heating medium passed therethrough in sufficient volume and at a sufficiently high temperature to promptly form a shell of coke on each agglomerate, and continuing the heating of the agglomerates until coking thereof is completed.
11. The method of producing coked agglomerates which comprises preparing and agglomerating an intimate mixture of zinciferous material and carbonaceous material capable when appropriately coked of producing coked agglomerates possessing satisfactory residue strength for vertical retort smelting, subjecting said agglomerates with a substantial moisture content to a coking operation in which the agglomerates are initially heated by direct contact with a gaseous heating medium passed therethrough in sufficient volume and at a sufficiently high temperature to promptly form a shell of coke on each agglomerate, and continuing the heating of the agglomerates until coking thereof is completed.
- 60 12. In the method of coking agglomerates containing an intimate admixture of zinciferous and carbonaceous reducing materials including a coking agent, the steps which comprise subjecting an upper section of a moving continuous column of the agglomer-

ates to intensive heat treatment adapted to form a shell of coke on each agglomerate in said upper section of the column in a short time interval to fix the shape of the agglomerates before they are softened and crushed by overhead agglomerates, and continuing the heat treatment operation of the partially coked agglomerates as they are progressively lowered in the column of moving agglomerates until their interiors are coked.

In testimony whereof I affix my signature.  
EARL H. BUNCE.

70

75

80

85

90

95

100

105

110

115

120

125

130